# EUROPEAN PATENT SPECIFICATION

(11) **EP 1 798 741 B1**
(45) Date of publication and mention of the grant of the patent: **26.01.2011**
(21) Application number: 06025718.5
(22) Date of filing: 12.12.2006
(51) Int. Cl.: H01C 7/112

(54) **Current/voltage nonlinear resistor**
Strom/Spannung nichtlinearer Widerstand
Résistance courant/tension non-linéaire

(30) Priority: 19.12.2005 JP 2005365084
(43) Date of publication of application: 20.06.2007
(73) Proprietor: KABUSHIKI KAISHA TOSHIBA, Tokyo 105-8001 (JP)
(72) Inventor: Andoh, Hideyasu c/o Intellectual Property Division, Minato-ku Tokyo 105-8001 (JP); Kasuga, Yasunori c/o Intellectual Property Division, Minato-ku Tokyo 105-8001 (JP)
(74) Representative: Kramer - Barske - Schmidtchen

(56) References cited:
- EP-A- 1 150 306
- EP-A1- 0 029 749
- EP-A2- 0 070 468

## Description

### BACKGROUND OF THE INVENTION

### 1. Field of the Invention

The present invention relates to a current/voltage nonlinear resistor whose main component is zinc oxide (ZnO), and more particularly relates to a current/voltage nonlinear resistor in which improvements have been made to the composition of sub-components contained in the main component.

### 2. Description of the Related Art

Overvoltage protection devices such as lightning arrestors and surge absorbers are commonly incorporated into power systems or electronic device circuitry. The purpose of these devices is to protect the power system or electronic device circuitry by removing any overvoltage that has been superimposed over the normal voltage. Current/voltage nonlinear resistors are frequently used for these overvoltage protection devices. A current/voltage nonlinear resistor is a resistor with the property of exhibiting substantially insulating characteristics at ordinary voltage, but exhibiting low resistance when overvoltage is applied.

A current/voltage nonlinear resistor is a ceramic element whose main component is zinc oxide (ZnO), and the following characteristics are required of such resistors. Naturally, the resistor must have nonlinear resistance characteristics, meaning that the resistance value varies greatly with changes in voltage, but also needs to have a long enough service life that no deterioration occurs when voltage is continuously applied over an extended period, energy capability characteristics that allow it to absorb lightning surges and switching surges without damage, and so forth. Also, current/voltage nonlinear resistors are seen to have a property whereby the resistance value drops when the temperature is higher. Consequently, thermal stability with respect to high temperature is also required.

The procedure for producing a current/voltage nonlinear resistor will now be described (see Japanese Patent Publication H4-25681). The raw materials of the current/voltage nonlinear resistor are such that zinc oxide (ZnO) is the main component, and Bi₂O₃, Co₂O₃, MnO, Sb₂O₃, and NiO are added as sub-components. These raw materials are thoroughly mixed along with water and a binder, then granulated with a spray dryer or the like, and these granules are molded and sintered to obtained a sinter. After this, the side faces of the sinter are coated with an insulating substance for preventing surface flashover, and this coating is heat treated to form a side face insulating layer. A current/voltage nonlinear resistor is produced by polishing the two end faces of the sinter and forming electrodes.

As demand for power and the need for stabilization have grown in recent years, reducing the size of power transmission and conversion devices has become a pressing concern. current/voltage nonlinear resistors whose main component is zinc oxide (ZnO) have been used in lightning arrestors (overvoltage protection devices) because of their excellent nonlinear resistance characteristics, but as the resistance value rises, fewer current/voltage nonlinear resistors are stacked in a lightning arrestor. In other words, increasing the resistance of a current/voltage nonlinear resistor is an essential technological key to achieving a lightning arrestor that is more compact. Also, increasing the nonlinear resistance characteristics of a current/voltage nonlinear resistor means lower the insulation layer of a power transmission and conversion system, and is therefore linked to making power transmission and conversion devices more compact.

A number of current/voltage nonlinear resistors with improved nonlinear resistance characteristics have been proposed in light of this situation. For instance, with the current/voltage nonlinear resistor disclosed in Japanese Laid-Open Patent Application 2001-307909, the amounts in which Bi₂O₃, Co₂O₃, MnO, Sb₂O₃, NiO, and other such sub-components are contained are limited, and the crystal phase of the Bi₂O₃ contained in a sinter whose main component is zinc oxide (ZnO) is also limited, which allows the resistance value to be raised and superior nonlinear resistance characteristics to be obtained.

With the technology disclosed in Japanese Patents 2,933,881, 2,940,486, and 3,165,410, a rare earth oxide is added to a current/voltage nonlinear resistor whose main component is zinc oxide (ZnO) and whose sub-components are Bi₂O₃, Co₂O₃, MnO, Sb₂O₃ and so forth, the result of which is that the resistance value is raised and characteristics are enhanced.

EP 1 150 306 A2 relates to a current/voltage non-linear resistor comprising a sintered body having ZnO as a main component, an electrode applied to a surface of the sintered body and an insulation material applied to another surface of the sintered body, said main component containing, as auxiliary components, Bi, Co, Mn, Sb, Ni and Al in the form of their oxides, wherein a Bi₂O₃ crystalline phase in said sintered body includes an α-Bi₂O₃ phase representing at least 80 % of the total Bi₂O₃ phase.

EP 0 029 749 A1 discloses a voltage-dependent resistor of the bulk-type, comprising a sintered body consisting essentially of, as a main constituent, zinc oxide and, as additives, Bi₂O₃), Co₂O₃, MnO₂, Sb₂O₃, Cr₂O₃, B₂O₃, at least one of Al₂O₃, Ga₂O₃, NiO and SiO₂, wherein electrodes are applied to opposite surfaces of said sintered body.

### SUMMARY OF THE INVENTION

Today, however, with the larger capacity of substations and the greater demand for underground substations, there is an increasingly great need for making power transmission and conversion devices smaller. Accordingly, the characteristics required of a current/voltage nonlinear resistor are at an even higher level, and with the prior art mentioned above, it is difficult to satisfy these requirements. More specifically, when the charging ratio (the voltage that is ordinarily applied to the current/voltage nonlinear resistor) was set high, a conventional current/voltage nonlinear resistor sometimes suffered severe deterioration, so that the service life was not long enough.

Also, a reduction in the size of power transmission and conversion devices extends to reducing the size of a lightning arrestor, of course, and the following problems have been indicated when the resistance of a current/voltage nonlinear resistor was raised due to making a lightning arrestor more compact. Because the amount of surge energy absorbed increases proportionally as the resistance of a current/ voltage nonlinear resistor is raised, the heating temperature is also raised by joule heat of the current/voltage nonlinear resistor when surge energy is absorbed.

As discussed above, because a current/voltage nonlinear resistor has a property whereby its resistance decreases as the temperature rises, if the temperature is too high, a drop in resistance occurs and there is greater current leakage. That is, since the decrease in the resistance of a current/voltage nonlinear resistor with increased resistance is greater when the temperature is raised, it has been indicated that there is a problem with thermal stability.

As a result, current of commercial frequency after the absorption of surge energy causes thermal runaway, and this increases unevenness of heating in the current/voltage nonlinear resistor. This invites an increase in thermal stress, which can lead to the breakdown of the current/voltage nonlinear resistor. Therefore, unless excellent thermal stability has been ensured, the resistance of the current/ voltage nonlinear resistor cannot be raised high enough, and it is difficult to reduce the size of a lightning arrestor.

The present invention was proposed in light of these problems, and it is an object thereof to provide a current/voltage nonlinear resistor with which the resistance value, nonlinear resistance characteristics, and thermal stability can be improved by specifying the compositional range of sub-components, and the size of a lightning arrestor can be reduced.

The present invention was conceived in an effort to achieve the stated object. According to the present invention, a current voltage nonlinear resistor includes a sinter, wherein said sinter consists essentially of zinc oxide (ZnO) as the main component and bismuth (Bi), cobalt (Co), manganese (Mn), antimony (Sb), nickel (Ni), gallium (Ga), and a rare earth element (R) as sub-components in proportions, calculated as Bi₂O₃, Co₂O₃, MnO, Sb₂O₃, NiO, Ga³⁺, and R₂O₃, of 0.3 to 1.5 mol% Bi₂O₃, 0.3 to 2.0 mol% Co₂O₃, 0.4 to 3.0 mol% MnO, 0.5 to 4.0 mol% Sb₂O₃, 0.5 to 4.0 mol% NiO, 0.0005 to 0.02 mol% Ga³⁺, and 0.05 to 1.0 mol% R₂O₃, wherein the current voltage nonlinear resistor is in the form of a disk, wherein the relationship between the added amount of Ga³⁺ and the diameter of the disk is such as claimed in claim 1.

With the present invention, the reason for specifying the sub-components to the above compositional ranges is that the inventors conducted various research into the compositions of current/voltage nonlinear resistors in an effort to achieved the above object, and as a result learned that keeping the proportions within the above ranges yields good resistance, nonlinear resistance characteristics, and thermal stability, and conversely that the above characteristics suffer when the proportions are outside the above ranges. Specifically, if the compositional proportions of the sub-components are kept within the above ranges, high resistance can be ensured and the nonlinear resistance characteristics and thermal stability are improved, and this makes it possible to attain the high level of characteristics required at the current time.

The present invention provides a current/voltage nonlinear resistor with which the sub-components, namely, bismuth (Bi), cobalt (Co), manganese (Mn), antimony (Sb), nickel (Ni), gallium (Ga), and a rare earth element (R), are contained in the compositional proportion ranges given above, and this affords excellent resistance, nonlinear resistance characteristics, and thermal stability, which in turn allows a current/voltage nonlinear resistor to be provided that can contribute to making lightning arrestors smaller.

### BRIEF DESCRIPTION OF THE DRAWINGS

FIG. 1 is a cross section of the current/voltage nonlinear resistor pertaining to the present invention; and
FIG. 2 is a graph of nonlinearity and the Ga³⁺ added amount coefficient A.

### DESCRIPTION OF THE PREFERRED EMBODIMENTS

Embodiments of the present invention will now be described in specific terms through reference to FIGS. 1 and 2 and Tables 1 to 5. Tables 1 to 5 show evaluation indicators and contained amounts of current/voltage nonlinear resistors produced with varying amounts of sub-components contained. Of the sample numbers given in the tables, those marked with an asterisk have sub-components that are outside the compositional ranges pertaining to the present invention, and are comparative samples produced for the sake of comparison. Those not marked with an asterisk, meanwhile, have sub-components within the compositional ranges corresponding to the present invention.

### (1) First Embodiment

A first embodiment related to the present invention will be described through reference to FIG. 1 and Tables 1 and 2. FIG. 1 is a cross section of the current/voltage nonlinear resistor pertaining to this embodiment.

### Constitution

In this embodiment, zinc oxide (ZnO) was used as the main component. Bismuth (Bi), cobalt (Co), manganese (Mn), antimony (Sb), nickel (Ni), and gallium (Ga), were used as sub-components, and the final amounts in which these were contained, calculated as Bi₂0₃, Co₂O₃, MnO, Sb₂0₃, NiO, and Ga³⁺ were within the following ranges.

The product contained 0.3 to 1.5 mol% Bi₂0₃, 0.3 to 2.0 mol% Co₂O₃, 0.4 to 3.0 mol% MnO, 0.5 to 4.0 mol% % Sb₂0₃, 0.5 to 4.0 mol% NiO, and 0.0005 to 0.02 mol% Ga³⁺.

Furthermore, at least one type of rare earth oxide (R) selected from about dysprosium (Dy), europium (Eu), erbium (Er), thulium (Tm), gadolinium (Gd), yttrium (Y), holmium (Ho), and ytterbium (Yb) were contained in an amount of 0.05 to 1.0 mol%, calculated as R₂O₃.

### Production Procedure

The procedure for producing the current/voltage nonlinear resistors pertaining to this embodiment and comparative samples will now be described in specific terms. Bi₂O₃, Co₂O₃, MnO, Sb₂O₃, NiO, Dy₂O₃, and Ga³⁺ or Al³⁺ were measured out as sub-components in specific amounts with respect to the ZnO main component such that the amounts in which the components were contained in the current/voltage nonlinear resistors ultimately obtained were as indicated for sample numbers 1 to 44 in Tables 1 and 2. These raw materials were mixed in a mixer along with water and an organic binder, and each slurry was adjusted to a uniform consistency. The Ga³⁺ or Al³⁺ here was added as a nitrate aqueous solution.

Next, each of the slurries thus obtained was spray granulated in a spray dryer to produce a granulated powder with a grain size of about 100 µm. The granulated powder thus obtained was put in a metal mold and pressed into a disk with a diameter of 125 mm and a thickness of 30 mm, and this molded disk was heated to 500°C to remove the organic binder that had been added.

After this, the disk was fired for 2 hours at 1100°C to obtain the sinter 1 shown in FIG. 1. The side faces of the sinter 1 were coated with an inorganic insulating substance, and these coatings were heat treated to form side face insulating layers 2. Finally, the upper and lower end faces of the sinter 1 provided with the side face insulating layers 2 were polished to a specific thickness, after which electrodes 3 were thermal sprayed onto the polished faces of the sinter 1 to produce a current/voltage nonlinear resistor.

### Evaluation of Resistance

The characteristics of the various current/voltage nonlinear resistors produced by the above procedure were evaluated as follows. First, the resistance of the current/voltage nonlinear resistor was evaluated by measuring the initial operating voltage of the current/voltage nonlinear resistor (the voltage when 1 mA of AC current was applied; V_{1mA}). The higher the initial operating voltage, the fewer current/voltage nonlinear resistors that need to be stacked in a lightning arrestor, so this voltage is effective as an index for ascertaining how compact a lightning arrestor can be made.

### Evaluation of Nonlinear Resistance Characteristics

The voltage when a 10 kA impulse current of 8 x 20 µs was applied (V_{10kA}) was measured, and the ratio of this to the initial operating voltage V_{1mA} (V_{10kA}/V_{1mA}) was evaluated as a nonlinearity coefficient. The smaller the value of this nonlinearity coefficient, the better the nonlinear resistance characteristics.

### Evaluation of thermal stability

The thermal stability of the current/voltage nonlinear resistor was evaluated by measuring the resistance leakage current when AC voltage that was 90% of the initial operating voltage was applied in a 200°C thermostatic tank. Specifically, the less leakage current at high temperature there is at 200°C, the better the thermal stability. The compositions of ten elements with each added component composition were measured, and the average thereof was used for the compositional value. The measurement results are given in Tables 1 and 2.

**Table 1**

| Sample number | Amourits of sub-components contained (mol%) | | | | | | | | Initial operating voltage (V_{1mA)} | Nonlinearity V_{10kA}/V_{1mA} | Leakage current at high temperature (mA) |
|---|---|---|---|---|---|---|---|---|---|---|---|
| | Bi₂O₃ | Sb₂O₃ | MnO | NiO | Co₂O₃ | Ga³⁺ | Al³⁺ | Dy₂O₃ | | | |
| 1* | 0.20 | 2.00 | 1.00 | 2.00 | 1.00' | 0.003 | 0 | 0.50 | 813 | 1.560 | 25.0 |
| 2 | 0.30 | 2.00 | 1.00 | 2.00 | 1.00 | 0.003 | 0 | 0.50 | 625 | 1.453 | 13.4 |
| 3 | 0.50 | 2.00 | 1.00 | 2.00 | 1.00 | 0.003 | 0 | 0.50 | 552 | 1.458 | 10.3 |
| 4 | 1.00 | 2.00 | 1.00 | 2.00 | 1.00 | 0.003 | 0 | 0:50 | 498 | 1.467 | 9.7 |
| 5 | 1.50 | 2.00 | 1.00 | 2.00 | 1.00 | 0.003 | 0 | 0.50 | 405 | 1.472 | 8.9 |
| 6* | 1.80 | 2.00 | 1.00 | 2.00 | 1.00 | 0.003 | 0 | 0.50 | 350 | 1.492 | 8.0 |
| 7* | 0.50 | 0.30 | 1.00 | 2.00 | 1.00 | 0.003 | 0 | 0.50 | 368 | 1.502 | 7.4 |
| 8 | 0.50 | 0.50 | 1.00 | 2.00 | 1.00 | 0.003 | 0 | 0.50 | 402 | 1.475 | 8.9 |
| 9 | 0.50 | 1.00 | 1.00 | 2.00 | 1.00 | 0.003 | 0 | 0.50 | 502 | 1.462 | 9.2 |
| 10 | 0.50 | 3.00 | 1.00 | 2.00 | 1.00 | 0.003 | 0 | 0.50 | 598 | 1.468 | 11.2 |
| 11 | 0.50 | 4.00 | 1.00 | 2.00 | 1.00 | 0.003 | 0 | 0.50 | 605 | 1.487 | 13.5 |
| 12* | 0.50 | 5.00 | 1.00 | 2.00 | 1.00 | 0.003 | 0 | 0.50 | 698 | 1.521 | 16.5 |
| 13* | 0.50 | 2.00 | 0.20 | 2.00 | 1.00 | 0.003 | 0 | 0.50 | 444 | 1.524 | 8.7 |
| 14 | 0.50 | 2.00 | 0.40 | 2.00 | 1.00 | 0.003 | 0 | 0.50 | 478 | 1.492 | 9.1 |
| 15 | 0.50 | 2.00 | 0.80 | 2.00 | 1.00 | 0.003 | 0 | 0.50 | 542 | 1.458 | 9.2 |
| 16 | 0.50 | 2.00 | 2.00 | 2.00 | 1.00 | 0.003 | 0 | 0.50 | 578 | 1.472 | 9.1 |
| 17 | 0.50 | 2.00 | 3.00 | 2.00 | 1.00 | 0.003 | 0 | 0.50 | 595 | 1.482 | 11.5 |
| 18* | 0.50 | 2.00 | 4.00 | 2.00 | 1.00 | 0.003 | 0 | 0.50 | 602 | 1.542 | 14.8 |
| 19* | 0.50 | 2.00 | 1.00 | 0.30 | 1.00 | 0.003 | 0 | 0.50 | 395 | 1.501 | 9.8 |
| 20 | 0.50 | 2.00 | 1.00 | 0.50 | 1.00 | 0.003 | 0 | 0.50 | 488 | 1.492 | 8.2 |
| 21 | 0.5 | 2.00 | 1.00 | 1.00 | 1.00 | 0.003, | 0 | 0.50 | 502 | 1.472 | 9.2 |
| 22 | 0.50 | 2.00 | 1.00 | 3.00 | 1.00 | 0.003 | 0 | 0.50 | 580 | 1.443 | 11.2 |
| 23 | 0.50 | 2.00 | 1.00 | 4.00 | 1.00 | 0.003 | 0 | 0.50 | 602 | 1.440 | 13.5 |
| 24* | 0.50 | 2.00 | 1.00 | 5.00 | 1.00 | 0.003 | 0 | 0.50 | 621 | 1.502 | 17.9 |

**Table 2**

| Sample number | Amounts of sub-components contained (mol% | | | | | | | | Initial operating voltage V_{1mA} (V/mm). | Nonlinearity V_{10kA}/V_{1mA} | Leakage current at high temperature (mA) |
|---|---|---|---|---|---|---|---|---|---|---|---|
| | Bi₂O₃ | Sb₂O₃ | MnO | NiO | Co₂O₃ | Ga³⁺ | Al³⁺ | Dy₂O₃ | | | |
| 25* | 0.50 | 2.00 | 1.00 | 2.00 | 0.20 | 0.003 | 0 | 0.50 | 458 | 1.542 | 12.3 |
| 26 | 0.50 | | 1.00 | 2.00 | 0.30 | 0.003 | 0 | 0.50 | 498 | 1.490 | 9.2 |
| 27 | 0.50 | 2.00 | 1.00 | 2.00 | 0.50 | 0.003 | 0 | 0.50 | 524 | 1.462 | 9.2 |
| 28 | 0.50 | 2.00 | 1.00 | 2.00 | 1.50 | 0.003 | 0 | 0.50 | 575 | 1.442 | 11.2 |
| 29 | 0.50 | 2.00 | 1.00 | 2.00 | 2.00 | 0.003 | 0 | 0.50 | 592 | 1.432 | 13.5 |
| 30* | 0.50 | 2.00 | 1.00 | 2.00 | 2.50 | 0.003 | 0 | 0.50 | 618 | 1.502 | 21.5 |
| 31* | 0.50 | 2.00 | 1.00 | 2.00 | 1.00 | 0.0003 | 0 | 0.50 | 645 | 1.592 | 13.4 |
| 32 | 0.50 | 2.00 | 1.00 | 2.00 | 1.00 | 0.0005 | 0 | 0.50 | 618 | 1.472 | 19.9 |
| 33 | 0.50 | 2.00 | 1.00 | 2.00 | 1.00 | 0.001 | 0 | 0.50 | 584 | 1.468 | 10.9 |
| 34 | 0.50 | 2.00 | 1.00 | 2.00 | 1.00 | 0.005 | 0 | 0.50 | 542 | 1.460 | 9.9 |
| 35 | 0.50 | 2.00 | 1.00 | 2.00 | 1.00 | 0.01 | 0 | 0.50 | 51 | 1.490 | 9.7 |
| 36 | 0.50 | 2.00 | 1.00 | 2.00 | 1.00 | 0.02 | 0 | 0.50 | 495 | 1.497 | 11.2 |
| 37* | 0.50 | 2.00 | 1.00 | 2.00 | 1.00 | 0.03 | 0 | 0.50 | 46.2 | 1.582 | 10.9 |
| 38* | 0.50 | 2.00 | 1.00 | 2.00 | 1.00 | 0 | 0.003 | 0.50 | 552 | 1.459 | 18.2 |
| 39* | 0.50 | 2.00 | 1.00 | 2.00 | 1.00 | 0.003 | 0 | 0.03 | 342 | 1.502 | 7.2 |
| 40 | 0.50 | 2.00 | 1.00 | 2.00 | 1.00 | 0.003 | 0 | 0.05 | 443 | 1.495 | 8.1 |
| 41 | 0.50 | 2.00 | 1.00 | 2.00 | 1.00 | 0.003 | 0 | 0.10 | 492 | 1.482 | 9.2 |
| 42 | 0.50 | 2.00 | 1.00 | 2.00 | 1.00 | 0.003 | 0 | 0.30 | 524 | 1.462 | 9.9 |
| 43 | 0.5 | 2.00 | 1.00 | 2.00 | 1.00 | 0.003 | 0 | 0.100 | 59.1 | 1.489 | 12.5 |
| 44* | 0.50 | 2.00 | 1.00 | 2.00 | 1.00 | 0.003 | 0 | 1.50 | 594 | 1.524 | 20.1 |

As discussed above, the current/voltage nonlinear resistors with the sample numbers marked with an asterisk in Tables 1 and 2 had compositions outside the ranges of the present invention, and were samples produced for the sake of comparison. As is clear from the results in Tables 1 and 2, the characteristics of the comparative samples do not satisfy the conditions of an excellent current/voltage nonlinear resistor as specified above.
Initial operating voltage (V_{1mA}) > 400 V/mm
Nonlinearity coefficient (V_{10kA}/V_{1mA}) < 1.50
Leakage current at high temperature (200°C) < 15 mA

In contrast, the current/voltage nonlinear resistors with sample numbers not marked with an asterisk in Tables 1 and 2 were within the compositional ranges specified in the claims of the present invention, and therefore exhibited excellent results for initial operating voltage, nonlinearity coefficient, and leakage current at high temperature. Specifically, the current/voltage nonlinear resistors pertaining to this embodiment can be considered to have high resistance and excellent nonlinear resistance characteristics and thermal stability.

Let us now discuss the role of the various sub-components contained in this embodiment, and also mention that the characteristics of this embodiment are not attained with the comparative samples.

### Role of Bi₂O₃ (see Table 1)

Bi₂O₃ is a component that is present at the boundary of the zinc oxide (ZnO), which is the main component of the sinter, and is responsible for nonlinear resistance characteristics. The role of this component is to promote the growth of ZnO crystal grains. If we compare sample numbers 1 to 6 here, we see that when the amount of Bi₂O₃ was less than 0.3 mol% (sample number 1), the material was in the liquid phase during sintering, and the amount of Bi₂0₃ was inadequate to improve sintering.

Accordingly, excellent characteristics were not obtained in terms of nonlinearity and leakage current at high temperature. Also, when the amount of Bi₂O₃ was over 1.5 mol% (sample number 6), the growth of ZnO particles proceeded too much during sintering, so a sufficiently high initial operating voltage could not be obtained.

### Role of Sb₂O₃ (see Table 1)

Sb₂O₃ is a component that controls and makes uniform the growth of ZnO crystal grains during sintering by forming spinel (Zn₇Sb₂O₁₂) particles along with zinc oxide (ZnO). Its role is to improve nonlinear resistance characteristics and, at the same time, suppress the growth of ZnO crystal grains.

A comparison of sample numbers 3 and 7 to 12 reveals that if the Sb₂O₃ content is less than 0.5 mol% (sample number 7), there will be too few spinel particles capable of suppressing grain growth during sintering, so excellent characteristics cannot be obtained in terms of initial operating voltage and nonlinearity. If the amount of Sb₂O₃ is over 4 mol% (sample number 12), however, it will act as an insulating component in the sinter, and there will be too many spinel particles, so excellent characteristics cannot be obtained in terms of nonlinearity and leakage current at high temperature.

### Role of MnO (see Table 1)

MnO is a component that primarily forms a solid solution with spinel particles and improves nonlinear resistance characteristics. A comparison of sample numbers 3 and 13 to 18 reveals that if the MnO content is less than 0.4 mol% (sample number 13), the electrical characteristics are unstable at the ZnO grain boundary, so excellent nonlinearity cannot be obtained. If the amount of MnO is over 3 mol% (sample number 18), however, here again it is impossible to obtain excellent nonlinearity characteristics.

### Role of NiO (see Table 1)

NiO is similar to MnO in that it primarily forms a solid solution with spinel particles and improves nonlinear resistance characteristics. A comparison of sample numbers 3 and 19 to 24 reveals that if the NiO content is less than 0.5 mol% (sample number 19), the very little NiO will form a solid solution with the spinel particles, so excellent initial operating voltage and nonlinearity cannot be obtained. If the amount of NiO is over 4 mol% (sample number 24), however, the electrical characteristics are unstable at the ZnO grain boundary, so excellent nonlinearity characteristics and leakage current at high temperature characteristics cannot be obtained.

### Role of Co₂O₃ (see Table 2)

Co₂O₃ also is a component that primarily forms a solid solution with spinel particles and improves nonlinear resistance characteristics. A comparison of sample numbers 3 and 25 to 30 reveals that if the Co₂O₃ content is less than 0.3 mol% (sample number 25), the electrical characteristics are unstable at the ZnO grain boundary, so excellent nonlinearity cannot be obtained, but if the amount of Co₂O₃ is over 2 mol% (sample number 30), here again the electrical characteristics are unstable at the ZnO grain boundary, making it impossible to obtain excellent nonlinearity characteristics or leakage current at high temperature characteristics.

### Role of Ga³⁺ (see Table 2)

Ga³⁺ serves to improve nonlinear resistance characteristics by forming a solid solution in the ZnO particles and lowering the electrical resistance of the ZnO particles. Aluminum (Al) has often been used in prior art as a component with a similar purpose, but improving nonlinear resistance characteristics by adding gallium gives a current/voltage nonlinear resistor with better thermal stability than by adding aluminum.

A comparison of sample numbers 3 and 31 to 38 reveals that if the Ga³⁺ content is less than 0.0005 mol% (sample number 31), not enough Ga³⁺ will form a solid solution in the ZnO particles in the sinter, so the electrical resistance of the ZnO particles will be high and excellent nonlinearity cannot be obtained.

If the amount of Ga³⁺ is over 0.02 mol% (sample number 37), however, the Ga³⁺ will precipitate at the ZnO grain boundary and adversely affect the electrical characteristics of the ZnO grain boundary, so excellent nonlinearity cannot be obtained. Furthermore, compared to when Al³⁺ is added (sample number 38), adding Ga³⁺ allows better leakage current at high temperature characteristics to be obtained.

### Role of Dy₂O₃ (see Table 2)

If the above-mentioned Sb₂O₃, Co₂O₃, NiO, and MnO are added in too large an amount in an effort to raise the resistance of a current/voltage nonlinear resistor, the resistance value will be highly dependent on temperature, so thermal stability will decrease.

In view of this, in this embodiment, higher resistance is -achieved by adding Dy₂O₃, which is a rare earth oxide that has the effect of raising resistance, the added amounts of Sb₂O₃, Co₂O₃, NiO, and MnO are effectively reduced and the temperature dependence of resistance is thereby lessened, and the thermal stability of the current/voltage nonlinear resistor can be increased.

A comparison of sample numbers 3 and 39 to 44 reveals that if the Dy₂O₃ content is less than 0.3 mol% (sample number 39), there will not be enough Dy₂O₃ to have the effect of suppressing grain growth, so excellent initial operating voltage and nonlinearity cannot be obtained. If the amount of Dy₂O₃ is over 1.0 mol% (sample number 44), however, the electrical characteristics will be unstable at the ZnO grain boundary, making it impossible to obtain excellent characteristics in terms of nonlinearity or leakage current at high temperature.

Furthermore, an oxide of dysprosium (Dy) was used as a rare earth oxide in this embodiment, but oxides of other rare earth elements, namely, europium (Eu), erbium (Er), thulium (Tm), gadolinium (Gd), yttrium (Y), holmium (Ho), and ytterbium (Yb), may also be used, and these will have the same effect as an oxide of dysprosium (Dy). Also, as long as the amount in which the various rare earth oxides are contained ends up being within a range of 0.05 to 1.0 mol%, the combination thereof may be selected as desired.

As described above, in this embodiment zinc oxide (ZnO) is the main component and the final amounts of sub-components are within the ranges given above, which makes it possible to obtain a current/voltage nonlinear resistor that has high resistance and excellent thermal stability and nonlinear resistance characteristics. Accordingly, the number of stacked layers of current/voltage nonlinear resistor can be reduced while maintaining high reliability, and this contributes to making a lightning arrestor smaller.

### (2) Second Embodiment

### Constitution and Production Procedure

Next, a second embodiment related to the present invention will be described through reference to Table 3. This embodiment is characterized by being composed of a sinter containing 0.005 to 0.05 wt% silver (Ag), calculated as Ag₂O.

Specifically, Bi₂O₃ (0.5 mol%), Co₂O₃ (1.0 mol%), MnO (1.0 mol%), Sb₂O₃ (2 mol%), NiO (2 mol%), Dy₂O₃ (0.5 mol%), and Ga³⁺ (0.003 mol% as a nitrate aqueous solution) were measured out as sub-components in the final proportions given in parentheses above, and these components were added to the ZnO main component. Ag₂O was further added to this base composition so as to be contained in an amount of 0.001 to 0.1 wt%, and the current/voltage nonlinear resistors of sample numbers 45 to 50 shown in Table 3 were produced by the method described in the first embodiment above.

### Evaluation of Service Life Characteristics

The service life characteristics of these current/voltage nonlinear resistors were evaluated. This was accomplished by continuously applying the voltage (V_{1mA}) when a 1 mA current was flowing, in an air atmosphere at 120°C for 3000 hours, and measuring the percentage change in the leakage current (Iᵣ) before and after the application of V_{1mA}. The results are given in Table 3.

The percentage change here is expressed by the following formula. $\left({I}_{r} \left(after 3000 hours\right)-{I}_{r} \left(initial value\right)\right) / {I}_{r} \left(initial value\right) \times 100$

If the change in leakage current here is a negative value, this indicates that the current/voltage nonlinear resistor has excellent service life characteristics.

**Table 3**

| Sample number | Ag₂O content (wt%) | Percentage change in leakage, current (%) |
|---|---|---|
| 45* | 0.0001 | 9.2 |
| 46 | 0.005 | -1.2 |
| 47 | 0.010 | -5.4 |
| 48 | 0.020 | -9.2 |
| 49 | 0.050 | -0.6 |
| 50* | 0.100 | 4.9 |

### Effect

The current/voltage nonlinear resistors of sample numbers 45 and 50, which are marked with an asterisk in Table 3, have compositions outside the scope of the claims of the present invention. As is clear from the results given in Table 3, the characteristics of the comparative samples indicate that the percentage change in leakage current is a positive value, and the service life characteristics are low. In other words, when the added amount of silver, calculated as Ag₂O, was less than 0.005 wt%, there was no effect of improving service life characteristics. When the amount was over 0.05 wt%, though, this had the opposite effect of causing the service life characteristics to deteriorate.

In contrast, with this embodiment (sample numbers 46 to 49) in which the Ag₂O content was from 0.005 to 0.05 wt%, the percentage change in leakage current was a negative value (see Table 3), and it is clear that current/voltage nonlinear resistors with excellent service life characteristics were obtained.

Specifically, with this embodiment, adding silver in an amount of 0.005 to 0.05 wt%, calculated as Ag₂O, reduces the change over time in leakage current and improves the service life characteristics. Furthermore, in this embodiment, the effect of adding silver on the service life characteristics was only discussed for the base composition given in the Constitution and Production Procedure above, but the same effect will be obtained as long as the composition is within the range of the base composition given in Claim 1.

### (3) Third Embodiment

### Constitution and Production Procedure

Next, a third embodiment related to the present invention will be described through reference to Table 4. This embodiment is characterized by being composed of a sinter containing 0.005 to 0.05 wt% boron (B), calculated as B₂O₃.

Specifically, Bi₂O₃ (0.5 mol%), Co₂O₃ (1.0 mol%), MnO (1.0 mol%), Sb₂O₃ (2 mol%), NiO (2 mol %), Dy₂O₃ (0.5 mol %), and Ga³⁺ (0.003 mol% as a nitrate aqueous solution) were measured out as sub-components in the final proportions given in parentheses above, and these components were added to the ZnO main component. Up to this point this embodiment is the same as the second embodiment above.

B₂O₃ was further added to this base composition so as to be contained in an amount of 0.001 to 0.1 wt%, and the current/voltage nonlinear resistors of sample numbers 51 to 56 shown in Table 4 were produced by the method described in the first embodiment above. That is, in the third embodiment, B₂O₃ was contained, instead of the Ag₂O used in the second embodiment, in amounts between 0.001 and 0.1 wt%.

### Evaluation of Service Life Characteristics

The service life characteristics of these current/voltage nonlinear resistors were evaluated by the method given in the second embodiment. Table 4 shows the percentage change in leakage current in this third embodiment.

**Table 4**

| Sample number | B₂O₃ content (wt%) | Percentage change in leakage current (%) |
|---|---|---|
| 51* | 0.0001 | 9.8 |
| 52 | 0.005 | -21 |
| 53 | 0.010 | -3.5 |
| 54 | 0.020 | -8.2 |
| 55. | 0.050 | -6.9 |
| 56* | 0.100 | 12.5 |

### Effect

The current/voltage nonlinear resistors of sample numbers 51 and 56, which are marked with an asterisk in Table 4, have compositions outside the scope of the claims of the present invention. As shown in Table 4, the characteristics of the comparative samples indicate that the percentage change in leakage current is a positive value, and the service life characteristics are low.

In other words, the service life characteristics were low when the added amount of boron, calculated as B₂O₃, was less than 0.005 wt%, and when it was more than 0.05 wt%. In contrast, with this embodiment (sample numbers 52 to 55) in which the B₂O₃ content was from 0.005 to 0.05 wt%, the percentage change in leakage current was a negative value (see Table 4), and current/voltage nonlinear resistors with excellent service life characteristics were obtained.

Specifically, with this embodiment, adding boron in an amount of 0.005 to 0.05 wt%, calculated as B₂O₃, improves the service life characteristics, just as in the second embodiment. Furthermore, in this embodiment, the effect of adding boron on the service life characteristics was only discussed for the above-mentioned base composition, but the same effect will be obtained as long as the composition is within the range of the base composition given in Claim 1. Also, instead of adding silver or boron alone, both may be added at the same time, as long as the combined amount is between 0.005 and 0.05 wt%.

### (4) Fourth Embodiment

### Constitution and Production Procedure

A fourth embodiment related to the present invention will now be described. In this embodiment, Bi₂O₃ (0.5 mol%), Co₂O₃ (1.0 mol%), MnO (1.0 mol%), Sb₂0₃ (2 mol%), NiO (2 mol%), Dy₂0₃ (0.5 mol%), and Ga³⁺ (0.003 mol%) were measured out as sub-components in the final proportions given in parentheses above, these components were added to the ZnO main component, and current/voltage nonlinear resistors were produced by the method described in the first embodiment above. This embodiment is characterized in that Ga³⁺ is added as a nitrate aqueous solution.

### Evaluation of Resistance Stability

The stability of the resistance value is evaluated in this fourth embodiment. Specifically, the initial operating voltage (V_{1mA}) was measured for 100 current/voltage nonlinear resistors in which Ga³⁺ had been added as a nitrate aqueous solution, and the standard deviation of this initial operating voltage was calculated. As a comparative example, the initial operating voltage (V_{1mA}) was measured for 100 current/voltage nonlinear resistors in which Ga³⁺ had been added not as an aqueous solution, but as an oxide, and the standard deviation of this initial operating voltage was calculated.

### Effect

In this embodiment and the comparative example, the standard deviation was calculated, and as a result the standard deviation of V_{1mA} when the Ga³⁺ was added as a nitrate aqueous solution was 585, while the standard deviation of V_{1mA} when the Ga³⁺ was added as an oxide was 2406. Specifically, a current/voltage nonlinear resistor with vastly less variance in its characteristics could be obtained by adding the Ga³⁺ as a nitrate aqueous solution.

Because gallium (Ga) was added in an extremely small amount, when gallium oxide (Ga₂O₃), which is an oxide of gallium (Ga), was added, it was difficult to mix uniformly with the other raw materials, and there was a great deal of variance in the characteristics. In contrast, when gallium nitrate (Ga(N0₃)₃), which is a water-soluble gallium raw material, was added, it mixed as gallium ions with the other raw materials, which is believed to be why the characteristics were so stable.

### (5) Fifth Embodiment

### Constitution and Production Procedure

A fifth embodiment related to the present invention will be described through reference to Table 5. In this embodiment, Bi₂0₃ (0.5 mol%), Co₂O₃ (1.0 mol%), MnO (1.0 mol%), Sb₂0₃ (2 mol%), NiO (2 mol%), and Dy₂O₃ (0.5 mol%) were measured out as sub-components in the final proportions given in parentheses above, and these components were added to the ZnO main component.

Ga³⁺ was added as a nitrate, with the added amount varied, and the current/voltage nonlinear resistors of sample numbers 57 to 71 in Table 5 were produced by the method described in the first embodiment above. Here, the disk diameter of the current/voltage nonlinear resistors was either 35, 60, or 100 mm, and the added amount of Ga³⁺ was varied with the disk diameter.

The nonlinearity (V_{10kA}/V_{1mA}) of these current/voltage nonlinear resistors was evaluated by the method given in the first embodiment above, and the results are given in Table 5. The coefficient A in Table 5 is a coefficient in the following relational formula with the added amount of Ga³⁺.

This embodiment is characterized in that the above-mentioned coefficient A is between 5 and 14. $Added amount of {Ga}^{3 +} \left(mol%\right) = \left(A-0.042\times D\right) / 1000$
(A: coefficient; D: disk diameter (mm))

**Table 5**

| Sample number | D (mm) | Ga³⁺ added amount (mol%) | Coefficient A | Nonlinearity V_{10kA}/V_{1mA} |
|---|---|---|---|---|
| 57* | 35 | 0.002 | 3.47 | 1.742 |
| 58 | 35 | 0.004 | 5.47 | 1.672 |
| 59 | 35 | 0.008 | 9.47 | 1.652 |
| 60 | 35 | 0.12 | 13.47 | 1.672 |
| 61* | 35 | 0.015 | 16.47 | 1.729 |
| 62* | 60 | 0.002 | 4.52 | 1.568 |
| 63 | 60 | 0.003 | 5.52 | 1.502 |
| 64 | 60 | 0.005 | 7.52 | 1.492 |
| 65 | 60 | 0.01 | 12.52 | 1.502 |
| 66* | 60 | 0.013 | 15.52 | 1.584 |
| 67* | 100 | 0.0003 | 4.50 | 1.542 |
| 68 | 100 | 0.0008 | 5.00 | 1.468 |
| 69. | 100 | 0.003 | 7.20 | 1.458 |
| 70 | 100 | 0.008 | 12.20 | 1.468 |
| 71* | 100 | 0.012 | 16.20 | 1.521 |

### Effect

FIG. 2 shows the relation between the coefficient A and nonlinearity. As shown in FIG. 2, nonlinearity obviously varies with the amount in which gallium (Ga) is added. Here, when the current/voltage nonlinear resistor is disk shaped, added amount of gallium at which nonlinearity is good varies with the diameter of the disk. This is because the current density in the current/voltage nonlinear resistor varies with the disk diameter, and the optimal added amount of gallium is within the range of the relational formula given above.

In other words, as is clear from FIG. 2, if the coefficient A is between 5 and 14, this is the optimal region for obtaining excellent nonlinearity, regardless of the disk diameter of the current/voltage nonlinear resistor. This embodiment, in which Ga³⁺ is added in an amount at which the coefficient A will be from 5 to 14, allows exceedingly good nonlinear resistance characteristics to be obtained.

### (6) Other Embodiments

The present invention is not limited to the embodiments given above, and various modifications are possible as long as the sub-components bismuth (Bi), cobalt (Co), manganese (Mn), antimony (Sb), nickel (Ni), gallium (Ga), and a rare earth element (R), and silver (Ag) and boron (B) are within the compositional range given in the claims.

It is explicitly stated that all features disclosed in the description and/or the claims are intended to be disclosed separately and independently from each other for the purpose of original disclosure as well as for the purpose of restricting the claimed invention independent of the composition of the features in the embodiments and/or the claims. It is explicitly stated that all value ranges or indications of groups of entities disclose every possible intermediate value or intermediate entity for the purpose of original disclosure as well as for the purpose of restricting the claimed invention, in particular as limits of value ranges.

## Claims

1. A current/voltage nonlinear resistor including a sinter (1), said sinter consisting essentially of zinc oxide (ZnO) as the main component and bismuth (Bi), cobalt (Co), manganese (Mn), antimony (Sb), nickel (Ni), gallium (Ga), and a rare earth element (R) as sub-components,
wherein the sub-components, calculated as Bi₂O₃, Co₂O₃, MnO, Sb₂O₃, NiO, Ga³⁺, and R₂O₃, are contained in the following proportions:
Bi₂O₃: 0.3 to 1.5 mol%,
Co₂O₃: 0.3 to 2.0 mol%,
MnO: 0.4 to 3.0 mol%,
Sb₂O₃: 0.5 to 4.0 mol%,
NiO: 0.5 to 4.0 mol%,
Ga³⁺: 0.0005 to 0.02 mol%, and
R₂O₃: 0.05 to 1.0 mol%,
wherein the current/voltage nonlinear resistor is in the form of a disk, whereby the relationship between the added amount of Ga³⁺ and the diameter of the disk is such that
the added amount of Ga³⁺ (mol%) ≤ (A- 0.042 × D)/1000
(where A = 5 to 14, and D = the disk diameter (mm)).

2. The current/voltage nonlinear resistor according to Claim 1, wherein the sinter (1) further contains 0.005 to 0.05 wt% silver (Ag), calculated as Ag₂O₃.

3. The current/voltage nonlinear resistor according to Claim 1, wherein the sinter (1) further contains 0.005 to 0.05 wt% boron (B), calculated as B₂O₃.

4. The current/voltage nonlinear resistor according to any one of Claims 1 to 3, wherein (R) is at least one member of the group consisting of dysprosium (Dy), europium (Eu), erbium (Er), thulium (Tm), gadolinium (Gd), yttrium (Y), holmium (Ho), and ytterbium (Yb).

5. The current/voltage nonlinear resistor according to any one of Claims 1 to 4, wherein a water-soluble raw material is used as a gallium (Ga) addition raw material.

## Patentansprüche

1. Strom/Spannung-nichtlinearer Widerstand, der einen Sinterkörper (1) umfasst, wobei der Sinterkörper im Wesentlichen aus Zinkoxid (ZnO) als Hauptkomponente und Bismuth (Bi), Cobalt (Co), Mangan (Mn), Antimon (Sb), Nickel (Ni), Gallium (Ga) und einem Seltenerdelement (R) als Nebenkomponenten besteht,
wobei die Nebenkomponenten, berechnet als Bi₂O₃, Co₂O₃, MnO, Sb₂O₃, NiO, Ga³⁺ und R₂O₃, in den folgenden Anteilen enthalten sind:
Bi₂O₃: 0,3 bis 1,5 mol-%
Co₂O₃: 0,3 bis 2,0 mol-%
MnO: 0,4 bis 3,0 mol-%
Sb₂O₃: 0,5 bis 4,0 mol-%
NiO: 0,5 bis 4,0 mol-%
Ga³⁺: 0,0005 bis 0,02 mol-% und
R₂O₃: 0,05 bis 1,0 mol-%,
wobei der Strom/Spannung-nichtlineare Widerstand in der Form einer Scheibe vorliegt, wodurch die Beziehung zwischen der zugesetzten Ga³⁺-Menge und dem Durchmesser der Scheibe derart ist, dass
die zugesetzte Ga³⁺-Menge (mol-%) ≤ (A - 0,042 × D)/1000 ist
(wobei A = 5 bis 14 und D = Scheibendurchmesser (mm)).

2. Strom/Spannung-nichtlinearer Widerstand nach Anspruch 1, wobei der Sinterkörper (1) ferner 0,005 bis 0,05 Gew.-% Silber (Ag), berechnet als Ag₂O₃, enthält.

3. Strom/Spannung-nichtlinearer Widerstand nach Anspruch 1, wobei der Sinterkörper (1) ferner 0,005 bis 0,05 Gew.-% Bor (B), berechnet als B₂O₃, enthält.

4. Strom/Spannung-nichtlinearer Widerstand nach einem der Ansprüche 1 bis 3, wobei (R) mindestens ein Element der Gruppe, bestehend aus Dysprosium (Dy), Europium (Eu), Erbium (Er), Thulium (Tm), Gadolinium (Gd), Yttrium (Y), Holmium (Ho) und Ytterbium (Yb), ist.

5. Strom/Spannung-nichtlinearer Widerstand nach einem der Ansprüche 1 bis 4, wobei als zuzusetzendes Gallium (Ga)-Ausgangsmaterial ein wasserlösliches Ausgangsmaterial verwendet wird.

## Revendications

1. Résistance courant/tension non-linéaire comprenant une fritte (1), ladite fritte étant constituée essentiellement d'oxyde de zinc (ZnO) comme composant principal et de bismuth (Bi), de cobalt (Co), de manganèse (Mn), d'antimoine (Sb), de nickel (Ni), de gallium (Ga) et d'un élément de terre rare (R) comme sous-composants,
dans laquelle les sous-composants, calculés pour Bi₂O₃, Co₂O₃, MnO, Sb₂O₃, NiO, Ga³⁺, et R₂O₃, sont contenus dans les proportions suivantes :
Bi₂O_{3 :} 0,3 à 1,5% en mole,
Co₂O₃ : 0,3 to 2,0% en mole,
MnO : 0,4 à 3,0 % en mole,
Sb₂O₃ : 0,5 à 4,0 % en mole,
NiO : 0,5 à 4,0 % en mole,
Ga³⁺ : 0,0005 à 0,02 % en mole,
et R₂O₃ : 0,05 à 1,0% en mole,
dans laquelle la résistance courant/tension non-linéaire a la forme d'un disque,
la relation entre la quantité ajoutée de Ga³⁺ et le diamètre du disque étant telle que
la quantité ajoutée de Ga³⁺ (% en mole) ≤ (A - 0,042 x D) /1000 (où A = 5 à 14 et D = diamètre du disque (mm)).

2. Résistance courant/tension non linéaire selon la revendication 1, dans laquelle la fritte (1) contient en outre 0,005 à 0,05 % en poids d'argent (Ag), calculé pour Ag₂O₃.

3. Résistance courant/tension non linéaire selon la revendication 1, dans laquelle la fritte (1) contient en outre 0,005 à 0,05 % en poids de bore (B), calculé pour B₂O₃

4. Résistance courant/tension non linéaire selon l'une quelconque des revendications 1 à 3, dans laquelle (R) est au moins un élément du groupe constitué du dysprosium (Dy), de l'europium (Eu), de l'erbium (Er), du thulium (Tm), du gadolinium (Gd), de l'yttrium (Y), de l'holmium (Ho) et de l'ytterbium (Yb).

5. Résistance courant/tension non linéaire selon l'une quelconque des revendications 1 à 4, dans laquelle un matériau brut soluble dans l'eau est utilisé sous la forme d'un matériau brut additionnel de gallium (Ga).
